

# UNITED STATES PATENT OFFICE.

JOSEPH GUSTAVE STODOLA, OF AGRAM, AUSTRIA-HUNGARY, ASSIGNOR TO GUSTAV J. A. TROSTEL, OF MILWAUKEE, WISCONSIN.

## PROCESS OF TANNING.

1,167,951.

Specification of Letters Patent. Patented Jan. 11, 1916.

No Drawing.

Application filed March 12, 1909. Serial No. 482,920.

To all whom it may concern:

Be it known that I, JOSEPH GUSTAVE STODOLA, a subject of the Emperor of Austria-Hungary, residing at Agram, in the 5 Province of Croatia and Empire of Austria-Hungary, have invented a certain new and useful Process of Tanning, of which the following is a specification.

My invention or discovery provides a new 10 and useful process for tanning hides and skins by the use of iron and chromium compounds to produce durable leather. By the expression "durable leather" I mean leather which is so tanned that the action of water 15 does not wash out the tanning agent or agents, as distinguished from such leathers as the alum tanned leathers.

Chrome tanning methods are well known in the art, and are extensively used in the 20 production of leathers, but these methods are expensive not only on account of the comparatively high cost of the chromium salts employed, but also because the leather produced by these methods has a peculiar 25 greenish or bluish hue which must be concealed or disguised by dyes before the leather is acceptable to users.

Iron salts are cheap, and as they possess the property of tanning hides and skins, they 30 would make most desirable tanning agents, but unfortunately they produce a harsh leather which is not generally suitable for the uses to which leather is applied. I have discovered however, that the salts of iron 35 and chromium can be used together in such a manner in tanning hides and skins, that the resulting leather is as good and serviceable as chrome or vegetable tanned leather, and has a nice yellow or buff color, so that 40 it is acceptable to users without previous dyeing. By my discovery therefore, I am enabled to produce marketable leather at a lower cost for tanning agents than heretofore, and which requires no expense for dyes.

45 In this specification and the claims, the term "hides" is used generically to include all classes of hides, skins and pelts.

In tanning hides by my new and improved

process, it is possible to vary the steps of the process somewhat, and it is possible to 50 vary the proportions of the materials employed somewhat, and the steps of the process and the proportions of materials should be altered as required by existing conditions at different tanneries, these matters being 55 matters which the judgment and skill of the tanner must determine. Without therefore, specifically limiting my process to the exact succession of steps which I am about to describe, and to the exact proportions of materials which I am about to state, I describe now at length what I consider at the present time to be the most preferable process for using iron and chromium compounds in 60 tanning leathers, and this description gives 65 in exact sequence and in exact proportions, full and explicit instructions for tanning hides according to my new process, without however depriving me of the right to make 70 variations therein as required by special circumstances, or as may seem advisable under certain conditions.

The hides are treated in the usual preliminary ways known to all tanners, to accomplish the removal of salt, dirt, hair, etc., 75 as though they were to be tanned by any of the well known processes. They are also bated in the usual manner, and are then treated as follows; it being understood that the weight of hide to be tanned determines 80 the proportions of the agents specifically given for a certain weight of hides, and it should also be understood that when solutions are stated with proportions that give 85 a certain strength, the strength of such solutions may be varied, the amount of solution used being varied accordingly. For example, a solution of one half the strength of another may be employed, but twice as much of the weakened solution will be required, or 90 vice versa.

Starting with 300 parts by weight of bated hides, the hides are first covered with a pickling solution having the following composition, viz: 600 parts of water; 3.6 95 parts of commercial strong sulfuric acid

of 66° Baumé scale, and 30 parts of common salt. Preferably the white bated hides are placed in a drum together with this pickling solution, and drummed for one hour; then 5 they are allowed to rest in this pickling solution for a further period of twelve hours. As the result of this pickling process the hides should absorb approximately one per cent. (calculated on the weight of the bated 10 hides, or what is known to tanners as the white weight, so that the total weight of the bated hides and absorbed acid will be approximately 101 per cent. of the weight of the bated hides) of acid, calculated as sulfuric acid; that is to say, the one per cent. 15 of acid though consisting of sulfuric acid and muriatic acid, is calculated as though it were all one acid. Thereafter, as the preferable form of treatment, there is added to 20 the pickled hides, a one-bath chrome liquor such as is ordinarily used in making chrome tanned leathers, such as, for example, the liquor of the Dennis Patent No. 495,028 of April 11, 1893, or any similar and equivalent 25 liquor. The purpose of this is to give the white hides a preliminary chrome tannage. This preliminary chrome tannage I at present consider as the best method of proceeding in carrying out my process. Where 30 the chrome is added at this stage of the process, the amount of the one-bath chrome liquor to add depends on the kind of leather it is wished to produce, as when the quantity of chrome liquor is increased, the resulting leather is softer, and vice versa, so 35 the tanner can easily govern this in accordance with the results desired.

While I have stated the use of a one-bath chrome liquor for giving a preliminary chrome tannage, it is not to be understood that this preliminary chrome tannage by the one-bath chrome liquor excludes a preliminary chrome tannage by the ordinary two-bath chrome process, as one method is 40 the equivalent of the other as far as my new and improved process of tanning is concerned. Where however, the preliminary chrome tannage is given by the two-bath process, the hides or leather should first be 45 washed before proceeding with the subsequent steps of the process. In some two-bath chrome processes there is a large precipitation of sulfur and this sulfur would act detrimentally on the subsequent iron and chrome solution and the object of the 50 washing is to get rid of the sulfur as much as possible, but where the one-bath chrome process is used, there is no sulfur and no washing is required.

55 In describing my process I am following what seems to me to be the simplest way of explaining it so that it will be readily understood. As described heretofore, the white, bated hides are placed in a tanning

drum, for convenience of treatment, with 65 the pickling solution. The one-bath chrome liquor is added to the drum containing the hides and the residual pickling solution. The hides and these solutions constitute the 70 contents of the drum when the stock iron and chrome solution described in the next paragraph is added to the contents of the drum. If, however, the hides have been removed from the drum and washed as described in connection with the preliminary 75 tannage by some two-bath chrome processes, then the hides are put into the drum with water before the stock iron and chrome solution is added to the contents of the drum.

The hides are then drummed in a tanning 80 drum or treated by equivalent mechanism for a few hours, and then there is added to the contents of the drum, 34 parts of a stock iron and chrome solution which is hereinafter described, and the hides are 85 then drummed for several hours. The partially tanned hides are allowed to remain in this liquor over night or for an equivalent period of time, and the first thing in the morning there is again added a further 90 quantity of the stock iron and chrome solution which has first been treated in the following manner: 30 parts of the stock iron and chrome solution are treated with 72 parts of a stock alkali solution hereinafter 95 described, preferably carbonated alkali such as sodium carbonate. These solutions are mixed before being added to the liquor in which the hides are. When these two solutions are mixed, any precipitation caused 100 by the addition of the sodium carbonate should redissolve. The color of the liquor is changed by the sodium carbonate to a dark reddish brown. This new liquor formed by mixing the stock iron and chrome 105 solution and the stock alkali solution is then added to the liquor in the drum in which the hides have remained, and drumming is continued for a few hours. Then another mixture is prepared of the stock iron and 110 chrome solution and the stock alkali solution in the same proportions and in the same manner as already described, and is added to the liquor in the drum and drumming is continued for a few hours more. The hides 115 are allowed to remain in the liquor over night and all of the next day up to about four o'clock in the afternoon, or for an equivalent period of time. They are then removed and allowed to drain over night. 120 On the following day a solution of 6 parts of borax in 250 parts of water or other alkali solution of equivalent strength is prepared, and enough of this solution is used on the tanned leather so that the amount of 125 borax shall be two and one-half per cent. of the weight of the drained leather. The leather is drummed for three-quarters of an

hour in this solution, which is intended to prevent the iron washing out of the leather. The leather is then washed three times with lukewarm water in the wheel.

5 In case the preliminary tannage with chrome is not desirable, as this preliminary tannage is not necessary for certain kinds of leather, the preliminary tannage can be omitted and the process carried out in all 10 other respects as described.

The "certain kinds of leather" just referred to in the production of which the preliminary tannage with chrome is not desirable and can be omitted, are what are 15 known as the hard leathers, as for example, sole leather for shoes. The preliminary tannage with chrome produces what are known as soft leathers, which are used for the uppers of shoes, for gloves, &c., and in general 20 it may be stated that when the result desired is a soft leather, the preliminary tannage with chrome should be used, but when the result desired is a hard leather, the preliminary tannage with chrome can be 25 omitted.

The stock iron and chrome solution referred to herein may be prepared as follows: Place 800 parts of sulfate of iron ( $FeSO_4 \cdot 7H_2O$ ) in a spacious vessel, and add 30 lukewarm water enough to cover it. Then add while stirring, 280 parts of commercial sulfuric acid ( $H_2SO_4$ ). The mixture will heat up during this operation. Then add 280 parts of a solution of sodium bichromate ( $Na_2Cr_2O_7$ ) containing 33% of 35 chromic acid ( $CrO_3$ ). Enough bichromate should be used so that there will be a slight excess of bichromate in order to insure the complete oxidation of the iron. If on testing it is found that the iron is not fully oxidized, more bichromate should be added. Cool and let stand. Then add enough water 40 to make the total volume equal to 2000 parts.

45 Muriatic acid may be used in place of sulfuric acid, and perhaps other acids, but I have so far used sulfuric acid. Potassium bichromate, ammonia bichromate or commercial chromic acid may be used in place 50 of the sodium bichromate.

The reactions in preparing the stock iron and chrome solution may be represented by the following formula:



The stock alkali solution referred to herein, may be conveniently prepared as follows: 60 Take 53 parts by weight of pure carbonate of soda ( $Na_2CO_3$ ), and enough water to make the combined weight of soda and water 1000 parts. Soda ash may be used, or washing soda, in place of pure sodium

carbonate, using an amount in either case 65 that will contain 53 parts by weight of pure carbonate of soda. Where other alkalis are used, an amount is taken that will be the chemical equivalent in neutralizing power.

It will of course be understood that any 70 other basic solution of iron containing chromic oxid ( $Cr_2O_3$ ) may be used in place of the basic sulfate of iron described, as for example, the basic chlorid or nitrate of iron, or a basic sulfate containing substances to 75 prevent precipitation, such substances for example, being sugars.

The amounts of materials given in the formula for the stock iron and chrome solution can be varied in proportion to the 80 amount of leather being treated, as much less quantities can be used in proportion to the amount of leather being tanned where the amount of leather is large, than when the amount of leather is small. This question of proportion of solution varying with the amount of leather undergoing treatment, is one which is familiar to all tanners and need not be discussed here more at length.

When the one-bath, preliminary chrome 90 tanning has been employed it is not necessary to add the stock alkali solution to the first bath of stock iron and chrome solution because the liquor, after adding the stock iron and chrome solution, is basic and will 95 tan but after the hides have extracted some of the tanning material it is then desirable to add basic solutions of iron.

If the hides have been washed, as described in connection with the two-bath, preliminary chrome tanning, this washing will have removed the residual, basic chrome tanning solution and the treatment with the stock iron and chrome solution should commence with the stock iron and chrome solution which has first been treated with the stock alkali solution as hereinbefore described. The remainder of the treatment will then be as described in this specification.

What I claim is:

1. The process of tanning hides to produce durable leather which consists in subjecting them to the tanning action of both iron and chromium compounds.

2. The process of tanning hides which consists in subjecting the hides to the tanning action of basic iron salts and basic chromium compounds.

3. The process of tanning hides which consists in subjecting the hides to the tanning action of chromium compounds and then subjecting them to the combined action of basic chromium compounds and basic iron salts.

4. The process of tanning hides which 125 consists in subjecting them to pickling solution so that they will absorb acid, then treating them to a preliminary chrome tannage.

then treating them with basic iron salts and basic chromium compounds in the same solution.

5. The process of tanning hides which  
5 consists in subjecting them to a pickling so-  
lution so that they will absorb acid, then  
treating them to a preliminary chrome tan-  
nage, then treating them with basic iron  
salts and basic chromium compounds in the  
10 same solution, removing them from the so-

lution and permitting them to drain, then  
treating them in an alkali solution to pre-  
vent washing out much of the iron, and  
finally washing them with lukewarm water.

In witness whereof I hereto affix my sig- 15  
nature in presence of two witnesses.

JOSEPH GUSTAVE STODOLA.

Witnesses:

CHAS. L. GOSS,

FRANK E. DENNETT.